

# UNITED STATES PATENT OFFICE.

WILLIAM A. McADAMS, OF BAY SHORE, NEW YORK.

## ALUMINUM ALLOY.

1,247,977.

Specification of Letters Patent. Patented Nov. 27, 1917.

No Drawing. Application filed April 15, 1914, Serial No. 832,050. Renewed May 1, 1917. Serial No. 165,799.

*To all whom it may concern:*

Be it known that I, WILLIAM A. McADAMS, a citizen of the United States, and resident of Bay Shore, in the county of 5 Suffolk and State of New York, have invented a new and useful Improvement in Aluminum Alloys, of which the following is a specification.

My invention relates to an aluminum alloy, with the object in view of providing a superior alloy suitable for casting purposes, which will not tarnish and which will possess the qualities of great fluidity and strength.

With these ends in view, my invention consists in an alloy composed of aluminum, copper, zinc, antimony, and silver, in which, by weight, the amount of antimony exceeds the amount of silver, the amount of zinc exceeds the amount of antimony, the amount of copper exceeds the amount of zinc, and the amount of aluminum exceeds the amount of copper.

The aforesaid elements are preferably combined in the proportions of, one hundred parts by weight of aluminum, seventeen parts by weight of copper, five parts by weight of zinc, one and one-half parts by weight of antimony, and one part by weight of silver.

In making the alloy, the antimony is melted in about one quarter of the aluminum at a high heat. The copper is then added

and then the silver is added. The heat of the mass is then lowered and the balance of 35 aluminum is added. The mass is agitated thoroughly and the temperature still further lowered to a dull red and then the zinc is added.

The mass is still thoroughly agitated and 40 the scum removed and the mass may then be cast into ingots.

What I claim is:—

1. An aluminum alloy composed of aluminum, copper, zinc, antimony and silver, 45 in which, by weight, the amount of antimony exceeds the amount of silver, the amount of zinc exceeds the amount of antimony, the amount of copper exceeds the amount of zinc, and the amount of aluminum 50 exceeds the amount of copper.

2. An aluminum alloy composed of aluminum, copper, zinc, antimony and silver combined in substantially the following proportions by weight; aluminum, one hundred parts; copper, seventeen parts; zinc, five parts; antimony one and one-half parts; and silver, one part.

In testimony, that I claim the foregoing as my invention, I have signed my name 60 in the presence of two witnesses, this fourteenth day of April, 1914.

WILLIAM A. McADAMS.

Witnesses:

F. GEORGE BARRY,  
LIDA M. EGBERT.